

1

3,482,688

**PHOSPHATE FLOTATION PROCESS**

Charles H. G. Bushell, Montrose, British Columbia, and Horst E. Hirsch, Trail, British Columbia, Canada, assignors to Cominco Ltd., Montreal, Quebec, Canada, a corporation of Canada

No Drawing. Filed July 8, 1966, Ser. No. 563,662  
Int. Cl. B03d 1/02

U.S. Cl. 209—166

5 Claims

**ABSTRACT OF THE DISCLOSURE**

A process for beneficiating phosphate rocks high in silicates and calcium and magnesium carbonates comprising subjecting said materials in comminuted form to an anionic froth flotation in an aqueous solution of a soluble fluoride selected from the group consisting of ammonium, hydrogen, sodium and potassium fluoride in the presence of a fatty acid collector. The resulting products are a froth product containing magnesium and calcium carbonates and a phosphate-enriched underflow concentration product.

This invention relates to a process for the beneficiation of phosphate-bearing materials and is particularly directed to a flotation process for the concentration of phosphate minerals such as apatite in phosphate rock.

Phosphate rock used in the production of phosphoric acid and phosphate fertilizers has phosphate minerals which occur in a plurality of forms, the more common of which and most important commercially being apatite,  $\text{Ca}_5(\text{PO}_4)_3\text{F}$ , found normally in association with gangue minerals such as silicates, calcite, dolomite and magnesite. The silicate or silica constituent of the rock commonly is removed by subjecting the comminuted rock to a primary anionic flotation wherein the phosphate minerals are collected and concentrated as a forth product and the silica minerals depressed and removed in the underflow as tailings. The froth product may then be subjected to a cationic flotation wherein the residual silica in the primary froth product is collected in the second stage froth as tailings and the valuable phosphate minerals depressed and removed in the underflow as a concentrate product. The calcite, magnesite and dolomite in their respective forms as calcium and magnesium carbonates have flotation characteristics similar to that of the phosphate minerals resulting in the concentration of the carbonates with the phosphate minerals.

In that carbonates present in the phosphate concentrate preferentially react with sulphuric acid when the concentrate is used in the wet phosphoric acid process for the production of phosphoric acid, the carbonates present cause undesirable foaming in the reactor chambers with resulting interruption of the operation and undue consumption of the acids. Also, the magnesium present in the phosphate concentrate forms soluble salts which increase the viscosity of phosphoric acid, and cause other difficulties when the acid is ammoniated to produce ammonium phosphate fertilizers.

It is also known to use soluble alkaline phosphates at a pH between 6 and 7 in an anionic flotation system to separate calcium carbonate from phosphate minerals whereby the calcium carbonate is collected as tailing in the froth and the phosphate minerals are depressed and concentrated as product in the underflow. For example, United States Patent No. 3,113,838 issued Dec. 10, 1963, discloses a process wherein sulphuric acid is employed to attack a portion of the phosphate minerals in an ore to produce phosphoric acid for transformation of the calcium phosphate into a soluble phosphate. This prac-

2

tice has been found unsatisfactory in that excessive quantities of sulphuric acid are consumed by preferential reaction with the carbonates rather than the phosphates and, as a result of the acid attack, the characteristics of the ore are altered. Also, the silica and silicate minerals report with the phosphate minerals interfering with the subsequent operation of the wet phosphoric acid process.

We have found that the bulk of the magnesium and calcium carbonates can be removed from phosphate-bearing materials by anionic froth flotation of the comminuted material suspended in an aqueous solution of a soluble fluoride selected from the group consisting of ammonium, hydrogen, sodium and potassium fluorides in the presence of a fatty acid collector. The resulting products are a froth product containing magnesium and calcium carbonates and a  $\text{P}_2\text{O}_5$ -enriched underflow concentrate product.

It is an important object of the present invention, therefore, to provide a method of beneficiating comminuted phosphate rocks high in silicates and calcium and magnesium carbonates to produce a concentrate rich in phosphate minerals and relatively low in calcium and magnesium carbonates and gangue minerals.

It is another object of the present invention to provide a method of beneficiating phosphate rocks and concentrates of hard rock phosphates known as apatite and colophane, by anionic flotation.

These and other objects of the present invention and the manner in which they can be attained will become apparent from the following detailed description of the embodiments and examples of the process.

According to the process of the invention, the phosphate rock to be beneficiated preferably is subjected, after appropriate comminution, to a primary anionic flotation using fatty acid collector reagents such as oleic acid, stearic acid, tall oils and the like to provide an enriched phosphate concentrate containing calcium and magnesium carbonates as a froth product and a silica tail as an underflow depressed product.

The phosphate-enriched froth concentrate is then subjected to an anionic flotation in an aqueous solution of a soluble fluoride present in amount of from about 1 to about 10 g.p.l., said solution having a pH within the range of from about 4.5 to about 7, preferably within the range of 5.8 to 6. The soluble fluoride can be selected from the group consisting of ammonium, hydrogen, sodium and potassium fluorides. The pH control can be maintained by the introduction to the solution of, for example, hydrofluoric acid, ammonium hydroxide and ammonia. The anionic collector may be a fatty acid selected from the group consisting of oleic acid, stearic acid, tall oil and the like.

The following examples show the effectiveness of the present process in the treatment of a colophane rock concentrate, colophane being a micro- or crypto-crystalline form of apatite. These examples are furnished for purposes of illustration only and it will be understood that the examples will not be construed as placing any limitations on the scope of the invention than as appears in the appended claims.

**EXAMPLE 1**

In this example of the process of our invention a primary phosphate concentrate feed containing 30.3%  $\text{P}_2\text{O}_5$ , 45.5%  $\text{CaO}$ , 0.9%  $\text{MgO}$  and 10.6%  $\text{SiO}_2$  and ground to pass 100 mesh was suspended in an aqueous solution containing 5.0 g.p.l. of ammonium acid fluoride ( $\text{NH}_4\text{F}\cdot\text{HF}$ ). The suspension was adjusted to contain approximately 30 to 35% solids and the pH adjusted to 5.8-6.0 using  $\text{NH}_4\text{OH}$  or HF as required. The suspension was then subjected to flotation using a fatty acid flotation reagent.

Table I below gives the results of this test:

anionic flotation which comprises suspending said phos-

TABLE I.—DEPORTMENT OF CaO, MgO, P<sub>2</sub>O<sub>5</sub> AND SiO<sub>2</sub>

| Float No.:     | NH <sub>4</sub> F-HF<br>in pulp,<br>g.p.l. | pH      | Fatty Acid<br>lb./ton<br>(accumul.) | Assays, percent               |      |      |                  | Distribution, percent (accum. floats) |      |                               |      |      |      |      |
|----------------|--------------------------------------------|---------|-------------------------------------|-------------------------------|------|------|------------------|---------------------------------------|------|-------------------------------|------|------|------|------|
|                |                                            |         |                                     | P <sub>2</sub> O <sub>5</sub> | CaO  | MgO  | SiO <sub>2</sub> | IL*                                   | Wt.  | P <sub>2</sub> O <sub>5</sub> | CaO  | MgO  |      |      |
| 1.....         | 5.0                                        | 5.8-6.0 | 0.52                                | 11.4                          | 36.3 | 12.0 | 6.0              | 29.3                                  | 3.7  | 1.4                           | 2.9  | 49.5 | 2.1  | 23.7 |
| 2.....         |                                            |         | 1.56                                | 25.5                          | 44.3 | 2.7  | 7.9              | 11.6                                  | 9.8  | 6.6                           | 9.2  | 68.1 | 6.7  | 39.4 |
| 3.....         |                                            |         | 3.11                                | 27.0                          | 43.5 | 1.8  | 9.3              | 8.7                                   | 10.8 | 7.4                           | 10.1 | 70.0 | 7.5  | 41.2 |
| Underflow..... |                                            |         |                                     | 31.4                          | 45.8 | 0.3  | 11.0             | 3.0                                   | 89.2 | 92.6                          | 89.9 | 30.0 | 92.5 | 58.8 |
| Feed.....      |                                            |         |                                     | 30.3                          | 45.5 | 0.9  | 10.6             | 4.6                                   | 100  | 100                           | 100  | 100  | 100  | 100  |

\*IL means Ignition Loss and is a measure of the CO<sub>2</sub> plus other volatile constituents, notably H<sub>2</sub>O.

In this example the float products 1, 2 and 3 account for 10.8% by weight of the feed and collectively account for 70% of the original MgO together with smaller amounts of CaO and SiO<sub>2</sub>. The concentrates, shown as the "underflow," account for 89.2% by weight of the feed and contain 31.4% P<sub>2</sub>O<sub>5</sub>, 45.8% CaO, 0.3% MgO and 11.0% SiO<sub>2</sub>.

#### EXAMPLE 2

A primary phosphate concentrate feed similar to that used in Example 1 was subjected to anionic flotation in aqueous solution containing 5.0 and 2.0 g.p.l. of sodium fluoride. The suspensions were adjusted to contain 30 to 35% solids and the pH adjusted to 5.8 to 6.0 by the introduction of hydrofluoric acid (HF). The suspensions were subjected to flotation using a fatty acid flotation reagent. Tables II(a) and II(b) below provide the results of this example.

TABLE II(a).—REFLOTATION OF PRIMARY PHOSPHATE CONCENTRATE IN NaF PULPS

| Float No.      | NaF<br>in<br>pulp,<br>g.p.l. | pH      | Fatty Acid<br>lb./ton<br>(accumul.) | Assays, percent               |      |     | Distribution, percent<br>(accum. floats) |                               |      |      |      |
|----------------|------------------------------|---------|-------------------------------------|-------------------------------|------|-----|------------------------------------------|-------------------------------|------|------|------|
|                |                              |         |                                     | P <sub>2</sub> O <sub>5</sub> | MgO  | IL* | Wt.                                      | P <sub>2</sub> O <sub>5</sub> | MgO  | IL*  |      |
| 1.....         | 5.0                          | 5.8-6.0 | HF                                  | 0.52                          | 25.5 | 3.5 | 12.9                                     | 3.7                           | 3.2  | 16.3 | 9.7  |
| 2.....         |                              |         |                                     | 1.56                          | 12.8 | 8.5 | 27.1                                     | 7.1                           | 4.6  | 52.2 | 28.2 |
| 3.....         |                              |         |                                     | 3.12                          | 22.2 | 3.0 | 12.8                                     | 14.1                          | 9.8  | 78.5 | 46.3 |
| Underflow..... |                              |         |                                     |                               | 31.5 | 0.2 | 3.1                                      | 85.9                          | 90.2 | 21.5 | 53.7 |
| Feed.....      |                              |         |                                     |                               | 30.0 | 0.8 | 5.0                                      | 100                           | 100  | 100  | 100  |

\* IL means Ignition Loss and is a measure of the CO<sub>2</sub> plus other volatile constituents, notably H<sub>2</sub>O.

TABLE II(b).—REFLOTATION OF PRIMARY PHOSPHATE CONCENTRATE IN NaF PULPS

| Float No.      | NaF<br>in<br>pulp,<br>g.p.l. | pH      | Fatty Acid<br>lb./ton<br>(accumul.) | Assays, percent               |      |     | Distribution, percent<br>(accum. floats) |                               |      |      |      |
|----------------|------------------------------|---------|-------------------------------------|-------------------------------|------|-----|------------------------------------------|-------------------------------|------|------|------|
|                |                              |         |                                     | P <sub>2</sub> O <sub>5</sub> | MgO  | IL* | Wt.                                      | P <sub>2</sub> O <sub>5</sub> | MgO  | IL*  |      |
| 1.....         | 2.0                          | 5.8-6.0 | HF                                  | 0.84                          | 19.4 | 7.0 | 19.7                                     | 3.4                           | 2.2  | 27.2 | 12.7 |
| 2.....         |                              |         |                                     | 2.40                          | 17.0 | 6.0 | 20.8                                     | 8.1                           | 4.9  | 60.0 | 31.5 |
| 3.....         |                              |         |                                     | 4.48                          | 25.5 | 1.9 | 10.2                                     | 12.8                          | 8.9  | 70.1 | 40.5 |
| Underflow..... |                              |         |                                     |                               | 31.4 | 0.3 | 3.6                                      | 87.2                          | 91.1 | 29.9 | 59.5 |
| Feed.....      |                              |         |                                     |                               | 30.0 | 0.9 | 5.3                                      | 100                           | 100  | 100  | 100  |

\* IL means Ignition Loss and is a measure of the CO<sub>2</sub> plus other volatile constituents, notably H<sub>2</sub>O.

In Table II(a) 78.5% by weight of the MgO contained in the original feed was rejected in the float, and in Table II(b), 70.1% of the MgO was rejected.

The present invention provides a number of important advantages. Siliceous phosphate rock can be beneficiated with a low consumption of additives and efficient removal of carbonates, especially magnesium containing carbonates. Phosphoric acid having a low magnesium salt content and suitable for the production of high quality phosphate fertilizers can be produced from this phosphate concentrate.

What we claim as new and desire to protect by Letters Patent of the United States is:

1. A process for beneficiating phosphate-bearing material containing apatite and calcium and magnesium carbonates comminuted for the substantial liberation of phosphate minerals from calcium and magnesium carbonate minerals and concentrated as a froth product by primary

phosphate-bearing material in an aqueous solution of a soluble fluoride selected from the group consisting of ammonium, hydrogen, sodium and potassium fluorides, adjusting the pH of said aqueous solution within the range of from about 4.5 to about 7, adding a flotation collector for the calcium and magnesium carbonate minerals, subjecting the mixture to froth flotation, and withdrawing an overflow product containing said carbonate minerals and an underflow product comprising a P<sub>2</sub>O<sub>5</sub>-enriched concentrate.

2. In a process as claimed in claim 1, said soluble fluoride having a concentration in said aqueous solution of at least 1 g.p.l.

3. In a process as claimed in claim 1, said soluble fluoride having a concentration in said aqueous solution within the range of from about 1 g.p.l. to about 10 g.p.l.

4. In a process as claimed in claim 3, adjusting the pH

of said aqueous solution within the range of from about 5.8 to about 6.

5. A process for producing a phosphate concentrate relatively low in magnesium content from phosphate bearing materials containing calcium and magnesium carbonates and silica which comprises the steps of subjecting said phosphate bearing material in finely divided form to

a primary anionic flotation operation, separately withdrawing from said primary flotation operation an underflow tailings product high in silica content and a phosphate enriched float product containing calcium and magnesium carbonates, suspending said phosphate enriched float product in an aqueous solution of a soluble fluoride selected from the group consisting of ammonium, hydrogen, sodium and potassium fluorides, adding to the resultant suspension a fatty acid flotation reagent, subjecting the suspension to a secondary anionic flotation operation, and withdrawing from said secondary flotation operation

70

an overflow product relatively high in calcium and magnesium carbonate content and an underflow product comprising a phosphate concentrate relatively low in magnesium content.

## References Cited

## UNITED STATES PATENTS

2,373,688 4/1945 Keck ----- 209—166  
3,113,838 12/1963 Perri ----- 209—166 X

3,361,257 1/1968 Maseman ----- 209—166  
2,442,455 6/1948 Booth ----- 209—166  
3,259,242 7/1966 Snow ----- 209—166

## FOREIGN PATENTS

5 468,161 9/1950 Canada.

HARRY B. THORNTON, Primary Examiner

ROBERT HALPER, Assistant Examiner

UNITED STATES PATENT OFFICE  
CERTIFICATE OF CORRECTION

Patent No. 3,482,688

December 9, 1969

Charles H. G. Bushell et al.

It is certified that error appears in the above identified patent and that said Letters Patent are hereby corrected as shown below:

Column 4, line 61 and column 5, lines 3 and 4, "magnesium" should read -- calcium and magnesium carbonate --.

Signed and sealed this 29th day of December 1970.

(SEAL)

Attest:

Edward M. Fletcher, Jr.

Attesting Officer

WILLIAM E. SCHUYLER, JR.

Commissioner of Patents